

## UNITED STATES PATENT OFFICE

2,169,392

PROCESS FOR THE PRODUCTION OF CELLULO-  
SIC TEXTILE FABRICDonald H. Powers, Moorestown, N. J., and Onslow  
B. Hager, Philadelphia, Pa., assignors to Röhm  
& Haas Company, Philadelphia, Pa.No Drawing. Application May 1, 1937,  
Serial No. 140,170

6 Claims. (Cl. 91—70)

This invention relates to a process for the production of a cellulosic textile fabric which combines many of the desirable characteristics of linen and of wool. It also relates to the product obtained by the application of this process.

Many attempts have been made to produce linen fabrics suitable for dress goods and suitings which are resistant to creasing and crushing but thus far no really satisfactory fabric has been obtained. Cotton and other cellulosic fabrics have been treated with various other materials, notably solutions of cellulose in aqueous solutions of quaternary ammonium bases, for the purpose of producing a fabric similar to linen. They have also been treated with resins such as phenol-formaldehyde and urea-formaldehyde resins for the purpose of increasing their resistance to creasing.

We have now found that a fabric having the crush resistance and feel of wool combined with the absorbent power and "coolness" of linen can be obtained by treating a cotton fabric, which has been coated with cellulose, with a urea-formaldehyde resin in such manner that the resin penetrates both the fiber and cellulose coating. In this manner a suiting material can be made from cotton which has all the advantages of linen suitings and at the same time possesses the crush resistance and feel of wool. Thus, the cellulose coating imparts a finish and sheerness to the cotton and also eliminates the lint, thus resulting in a smooth, thready fabric. When this entire, coated fabric is then treated with the urea-formaldehyde resin, it becomes crush-resistant to a much greater extent than would the original cotton or an equivalent piece of linen goods under the same treatment. This is due to the fact that the original cotton fibers of the fabric have been enlarged by the coating of cellulose and since this coating is also absorbent it too can absorb the urea-formaldehyde solution. In this way each individual fiber of the original fabric after cellulose coating can absorb more urea-formaldehyde resin without having any substantial amount of it on the surface which would tend to bind both fibers and threads together thus yielding a harsh, stiff fabric. This hardness is undesirable in suiting material.

We have found, furthermore, that very light weight, cotton fabrics, such as organdies and lawns, can be rendered quite sheer and permanently crisp by first applying the cellulosic coating in the prescribed manner and then introducing into the thus coated fabrics a remarkable degree of resilience and resistance to creasing by

impregnating with the urea-formaldehyde resin. The crush resistance thus obtained is much greater than is obtained from an equivalent amount of resin applied to the fabric which has not been previously coated with cellulosic materials. 5

The fabric is usually so treated with the cellulose solution that it increases about five per cent. in weight. As the specific gravity of the cellulose coating and that of the original cotton fiber are about the same, this means an increase of five per cent. in the volume of each fiber and, since regenerated celluloses absorb greater quantities of resin than ordinary cellulose, there is a consequent increase of about eight per cent. in 15 the amount of urea-formaldehyde resin which it can absorb and retain within itself. On account of this increase in the volume of each fiber and more particularly because of the greater concentration of resin in a layer farther removed 20 from the axis of the fiber resulting in greater resistance to bending according to well known mechanical principles, the improvement in the crush resistance of the finished fabric is much greater than that obtained by treating the original cotton with urea-formaldehyde resins only. A cotton fabric treated with urea-formaldehyde resin and subsequently coated with cellulosic materials is inferior to that obtained as described above, and is of much less value as a suiting 30 material or dress fabric although distinctly superior to the original fabric having no chemical finish of any kind. When the fabric is first treated with resin and after treated with cellulose, the high alkalinity of the cellulose coating 35 solution removes an appreciable portion of the resin and deposits on the surface of the fiber a film which does not impart as desirable a crush resistance as is obtained by the herein described process. Consequently, by first treating 40 a fabric with a cellulose solution, removing the last traces of alkali from this coating solution, and then treating with the resin, an unusually attractive fabric is produced which is substantially non-shrinkable and non-crushing. 45

The new treatment, which consists in first applying the cellulose coating to the fibers and then impregnating them with urea-formaldehyde resin, yields a fabric which is far superior to the original fabric or to any obtained by the individual treatments. 50

Cellulosic yarns may also be improved by the same treatment, viz: First coating them with cellulose and then impregnating them with a urea-formaldehyde condensation product which 55

is subsequently hardened. In this case also, both fiber and coating are impregnated with the condensation product. Fabrics woven from such yarns have a much greater porosity and a much greater resistance to creasing than fabrics woven from the untreated yarns.

The cellulose coating may be pure cellulose as precipitated from a viscose or cuprammonium solution but we prefer to use solutions of cellulose in quaternary ammonium bases, particularly those which have a benzyl group such as trimethyl benzyl ammonium hydroxide and other similar bases described in U. S. Patent No. 2,009,-015, granted July 23, 1935. The coating may also be a cellulose ether such as hydroxyethyl cellulose, methyl cellulose, etc., but only those ethers are applicable which after application form coatings that are permeable to aqueous solutions, particularly to those of the urea-formaldehyde resin or the ingredients from which it is made.

In general the fibers are coated with cellulose by passing the fabric through a solution thereof in a quaternary ammonium base such as trimethyl benzyl ammonium hydroxide containing about four to eight per cent. of cellulose and squeezing it under such conditions that the fabric takes up about its own weight of solution. It is then dried to touch and run into a precipitating bath such as dilute acid, washed thoroughly and dried. When thoroughly dry, it is run through the impregnating solution which is usually a solution of dimethylol urea of twenty to thirty per cent. concentration or one containing the equivalent amounts of urea and formaldehyde and again squeezed so that it picks up about its own weight of the solution. Following this the fabric is dried and the resin cured by heating it for a short period of time at temperatures ranging from about 275° to 350° F.

Fabric treated in this way is much firmer, fuller and more absorbent. When made up into clothing, it gives a garment which on account of its "coolness" is very suitable for use in hot weather. It is also much more resistant to crushing than an untreated fabric.

The following examples are given by way of illustration but the invention is not limited to the exact details of time, temperature, concentration, etc., shown as it may otherwise be practiced within the scope of the appended claims.

#### Example 1

A 40 x 32 cotton Osnaburg is desized and run through a cellulose solution which contains about six per cent. cellulose. This solution is prepared by adding sufficient five per cent. caustic soda solution to a fifteen per cent. solution of cellulose in concentrated trimethyl benzyl ammonium hydroxide to dilute it to six per cent. cellulose content. After passing through this solution, the fabric is squeezed so that the amount of solution it has absorbed is ninety to one hundred per cent. of the dry weight of the fabric. It is then dried until it is dry to touch and run through a two per cent. sulfuric acid solution to precipitate the cellulose on the fiber following which it is washed, dried and passed through the impregnating solution. This solution contains thirty per cent. of dimethylol urea, one per cent. of di-ammonium phosphate as a catalyst for the re-sification of the dimethylol urea and 0.3 per cent. of dimethyl lauryl benzyl ammonium chloride as a wetting agent. After passing through this solution the fabric is again dried and the resin with which it has been impregnated is cured

by heating at 290° F. for ten minutes. The resulting material is soft and resilient and will retain its weight and appearance even after repeated washings. The individual fibers have a five per cent. greater diameter and the entire fabric is about twenty-five per cent. heavier. Its tensile strength has also been increased by about twenty per cent.

#### Example 2

A 35 x 25 Osnaburg was desized and passed through a solution containing eight per cent. of alkali-soluble hydroxy ethyl cellulose dissolved in a five per cent. solution of sodium hydroxide. After passing through this solution the fabric is squeezed so as to pick up approximately its own weight of solution, dried, slightly acidified with weak sulfuric acid, rinsed and dried. This fabric is then run through a solution prepared by mixing one part of urea with two parts of forty per cent. formaldehyde solution. This mixture is made slightly alkaline with hexylmethylenetetramine, boiled for three minutes, cooled and diluted with water so that the resulting solution contains twenty-five per cent. of resin. Before applying this solution to the fabric one-half per cent. of acetic acid is added. The fabric coated with the hydroxy ethyl cellulose is passed through this bath, hydro extracted and cured for ten minutes at 340° F., rinsed and dried. In this manner an absorbent, crush-resistant suiting material is obtained.

#### Example 3

A 136 x 96 cotton shirting material is run through a cuprammonium solution containing four per cent. of dissolved cellulose and squeezed so that it takes up approximately its own weight of solution. The cellulose is then precipitated by passing the fabric through a sodium sulfite solution and subsequently rinsing it with weak sulfuric acid, washed and dried. The fabric thus coated is run through a solution containing twenty per cent. of dimethylol urea and one per cent. of ammonium acetate. After squeezing so that the fabric takes up about its own weight of the solution, it is dried and heated for ten minutes at 290° F. to harden the resin. The resulting fabric makes a very attractive ladies' dress material having the properties of linen and resistance to mussing and crushing of wool.

#### Example 4

A 36 x 26 sheeting is run through a five per cent. solution of viscose, dried and passed into a precipitating bath containing two per cent. of sulfuric acid and two per cent. of sodium sulfate. It is then thoroughly rinsed, dried and passed through a solution containing thirty per cent. of dimethylol urea, one per cent. of acetic acid and one-half per cent. of dimethyl cetyl butyl ammonium chloride. The fabric is then dried and heated to 300° F. for ten minutes to harden the resin.

#### Example 5

A 76 x 72 lawn is passed through a four per cent. solution of cellulose in concentrated trimethyl benzyl ammonium hydroxide, squeezed free of excess liquid so as to retain approximately its own weight of solution, and dried by passing through a hot tenter frame. The dried fabric is then run through a two per cent. sulfuric acid solution to precipitate the cellulose and neutralize the excess alkalinity, squeezed, and

washed free of acid, dried and then run through a thirty per cent. solution of dimethylol urea containing four per cent. diammonium phosphate (based on the dimethylol urea). The fabric was 5 squeezed so as to allow an equal weight of liquid to be taken up, dried and the resin then cured by subjecting the fabric to 270° to 280° F. for four minutes. The resulting material is stiff, wiry and sheer with an unusual degree of resiliency considering its stiffness. The tensile 10 strength is increased by about twenty per cent. and the fibers are so set that shrinkage is reduced. The resulting finish is a greatly improved, stiff organdy finish.

15 In the foregoing examples cotton fabrics have been used for purposes of illustration but it is obvious to any one skilled in the art that linen, rayon, or combinations of these materials with each other or with cotton can be treated in a 20 similar way. While cellulose solutions are particularly suited for this work, it is obvious that alkali-soluble cellulose ethers are also suitable as they coat the fiber with an adsorbent film. For this purpose the alkali-soluble methyl cellulose or ethyl cellulose is suitable as well as the 25 alkali-soluble hydroxyethyl cellulose.

We claim:

1. The process of improving cellulosic fabrics and yarn which comprises applying to the fibers 30 thereof a coating of cellulosic material selected from the group consisting of cellulose and cellulose ethers permeable to aqueous solutions, impregnating the coated fibers with an aqueous solution of a hardenable urea-formaldehyde

product, drying and heating to harden the urea-formaldehyde product.

2. The process of improving cellulosic fabrics and yarn which comprises applying to the fibers thereof a coating of cellulose, impregnating the 5 coated fibers with an aqueous solution of a hardenable urea-formaldehyde product, drying and heating to harden the urea-formaldehyde product.

3. The process of improving cellulosic fabrics 10 and yarn which comprises applying to the fibers thereof a coating of an alkali-soluble cellulose ether, impregnating the coated fibers with an aqueous solution of a hardenable urea-formaldehyde product, drying and heating to harden the 15 urea-formaldehyde product.

4. The process of improving cellulosic fabrics and yarn which comprises passing them through a solution of cellulose in a quaternary ammonium hydroxide, drying and setting the cellulose on 20 the fibers by treatment with dilute acid, rinsing, drying, impregnating with an aqueous solution of dimethylol urea, drying and heating to convert the dimethylol urea to an insoluble resin.

5. A cellulosic fabric, the fibers of which carry 25 a coating of cellulose, both fiber and coating being impregnated with a urea-formaldehyde condensation product.

6. A cellulosic yarn, the fibers of which have 30 been coated with cellulose and subsequently impregnated with a urea-formaldehyde condensation product.

DONALD H. POWERS.  
ONSLAW B. HAGER.